

Patented May 15, 1928.

1,669,660

# UNITED STATES PATENT OFFICE.

J BIRCHARD GREEN, OF CHICAGO, ILLINOIS, ASSIGNOR TO CHICAGO STEEL AND WIRE COMPANY, OF CHICAGO, ILLINOIS, A CORPORATION OF ILLINOIS.

## WELDING ROD.

No Drawing.

Application filed March 19, 1926. Serial No. 96,064.

My invention has to do with filler rods which are used as electrodes in metallic arc welding, and is particularly concerned with the manner in which the surfaces of such 5 rods are treated in order to stabilize the arc.

In metallic arc welding, the working characteristics of any one type of electrode are subject to fairly wide variation, depending on the residual quantity of lime, a lubricant 10 used in wire drawing, that happens to be left on the finished wire or electrode. The lubrication of wire during drawing to prevent its breaking into small pieces instead of passing through the dies in long continuous 15 lengths, is a delicate thing. If the drawing of the wire must be made secondary to the leaving of a substantial quantity of the lime lubricant on the finished wire, the drawing cannot be accomplished with maximum 20 economy, and, conversely, if the quantity of residual lime is disregarded, the finished electrode will vary in its working characteristics, this lack of uniformity making it difficult to use and at times preventing 25 the welder from performing commercially acceptable work. Furthermore, if the finished electrode has been passed several times through the drawing dies, it is practically impossible to leave a substantial quantity of 30 lime on the finished wire. It is often desirable, and in the lighter sizes absolutely necessary, to pass the wire many times through the dies.

It is a well known fact that metals, known 35 as first class conductors, increase in electrical resistance as their temperature is elevated, while second class conductors, to which class lime belongs, decrease. It is easy to understand that at the extremely high temperatures of the metallic arc this effect becomes very pronounced, and this accounts 40 for the fact that the presence of some second class conductor is essential in connection with a metallic arc electrode if a commercially stable arc is to be produced.

It has been the practice to apply a substantial quantity of second class conducting material to the surfaces of electrodes, whereby to produce an electrode which is completely sheathed in a so-called flux coating. 50 When such a substantial quantity is applied, however, the electrodes dry slowly and during the drying process must be kept out of contact with each other or at least a poor 55 appearing product results and often one

which on account of wide variation in the quantity of flux at different points along the electrode gives a wide variation in working characteristics.

Full flux coatings may not only stabilize 60 the arc but in addition perform other functions as throwing the preponderance of heat to one pole or the other in direct current welding, as adding to or subtracting from the composition of the electrode passed 65 metal, as forming an insulating coating, advantages in welding at the bottom of deep narrow grooves, and the like.

One object of my invention is to provide a surface which produces practically the 70 maximum of arc stability but which does not provide for any other appreciable influence on the arc or the deposit as is possible with a full flux coating.

Another object is to provide a method of 75 manufacture which will permit standardization of the electrode working characteristics so far as the stabilizing effect of surface materials is concerned without substantially increasing the cost of the electrodes over 80 that of so-called bare electrodes.

Another object is to improve the working characteristics of the electrodes without substantially increasing their cost of manufacture. 85

I have discovered that by eliminating consideration of the quantity of residual lime in the wire drawing, and applying a thin film of a second class conductor as a separate operation after the wire reaches finished 90 size, the quantity of such second class conductor can readily be controlled and standardized; that the electrodes can readily be so treated in mass during both dipping and drying that this can be accomplished and still apply a somewhat thicker film than the maximum possible as a residual coating of lime left after wire drawing. I find that the arc from electrodes treated in this manner is almost as stable as with a full flux coating; in fact, they can readily be used 95 for metallic arc welding with an alternating sixty cycle current source, which is not considered practical with the ordinary bare electrode.

Electrodes made by my method can be produced as cheaply as bare electrodes because the cost of applying the second class conductor is offset, or may be more than offset, by the economies possible in the wire 100 105 110

drawing, and more especially in the avoidance of rejections of electrodes too free from residual lime to give a commercially stable arc. Another advantage of my method is that it permits latitude in the selection of second class conductors while any that are left residual from wire drawing must primarily be proper wire mill lubricants. The most suitable second class conductors from the standpoint of stabilizing the arc seem to fall in the class of the more stable salts, oxides and hydroxides of the alkaline earths and metals. The lime left on the wire after drawing air slakes in a comparatively short time and becomes essentially calcium carbonate. Partly because of this which means that the welding industry has had long experience with its use in the small quantities present on bare electrodes, and partly on account of its cheapness and ease in handling, I prefer to use calcium carbonate in my method of surfacing electrodes.

Both lime and calcium carbonate are quite opaque, or have, what painters call, good covering power. On this account it is difficult to tell by inspection small differences in the thickness of the surface covering, especially if this be thin, and yet such small differences result in a substantial difference in the welding characteristics of electrodes. This permits confusion in a wire mill where electrodes are made by my method and other bare electrodes or other similarly drawn wires are made, and this is especially true if the quantity of residual lime is large and the finished wire has been wet with water. Confusion can also occur in the hands of the user of electrodes. To overcome this I precipitate a small amount of some pigment, neutral so far as welding is concerned in the quantity used, on the calcium carbonate used in connection with my method of surfacing electrodes. This alone might not always suffice because flux coatings have been pigmented, so I have selected the color green because to the best of my knowledge and belief

this has never been used to distinguish any electrode coating.

In order to make the electrode surfacing contemplated by my method adherent, I use an adhesive neutral in the quantity employed to welding. I have for this purpose used both soap and sodium silicate successfully. On account of ease of handling and cheapness I prefer sodium silicate. 55

Using the ingredients above described I find that the following formula gives a maximum thickness to the surfacing possible by my method of treating the electrodes in mass. Water, 500 parts by weight; calcium carbonate, 325 parts by weight; green pigment, 25 parts by weight; adhesive, to suit.

Definite proportion of the adhesive cannot be specified because of the variable nature of both soap and sodium silicate. So little, however, should be used as to leave the finished electrode what might be termed slightly dusty, i. e. the pigmented calcium carbonate should not be glazed on the surface because adhesive in such quantity might influence welding. 65 70

I claim:

1. A process of coating welding rods which comprises dipping the rods in a bath comprising about 500 parts of water, about 75 325 parts of calcium carbonate, about 25 parts of a green pigment and a suitable amount of adhesive to give the desired consistency.

2. A process of coating welding rods 80 which comprises dipping the rods in a bath containing a binder and about 325 parts of calcium carbonate to every 500 parts of water.

3. Welding rods having a weld-assisting 85 coating resulting from being dipped in a bath containing a binder and about 325 parts of calcium carbonate to every 500 parts of water.

In testimony whereof I have hereunto 90 subscribed my name.

J BIRCHARD GREEN.